

## UNITED STATES PATENT OFFICE

2,603,637

PREPARATION OF ORGANIC ACID ESTERS  
OF CELLULOSE

Peter Blackman, Westfield, and Fred Fortress and  
Blanche B. White, Summit, N. J., assignors to  
Celanese Corporation of America, New York,  
N. Y., a corporation of Delaware

No Drawing. Application May 18, 1950,  
Serial No. 162,826

13 Claims. (Cl. 260—229)

1

This invention relates to the preparation of organic acid esters of cellulose and relates more particularly to an improved process for the treatment of cellulosic material that is to be employed for the production of organic acid esters of cellulose.

In the production of organic acid esters of cellulose from cellulosic material, it is the general practice to pretreat the cellulosic material prior to esterification to increase its reactivity. The pretreated cellulosic material is then esterified with an organic acid anhydride, usually in the presence of an esterification catalyst, such as sulfuric acid, and an organic acid, such as acetic acid, which acts as a solvent for the cellulose ester being formed. The pretreatment of the cellulosic material greatly reduces the time required for the esterification. However, the pretreatment does not always impart the same reactivity to different batches of cellulosic material from a given source so that the time required for their esterification will vary appreciably. While provision can be made in a batch esterification process to adjust the esterification time in accordance with changes in the reactivity of the cellulosic material, there is an additional expense involved in making this adjustment. In a continuous process, on the other hand, the esterification time cannot be adjusted readily in accordance with changes in the reactivity of the cellulosic material. It is, accordingly, necessary, in a continuous process, to provide a sufficient esterification time to complete the esterification of the least reactive cellulosic material. As will be readily apparent, this increase in the time provided for esterification will reduce the capacity of the esterification equipment and increase the esterification cost.

Not only does the pretreatment fail to impart the same reactivity to different batches of cellulosic material from a given source, but it also fails to impart the same reactivity to all the cellulosic material in a single batch. That portion of the cellulosic material in a single batch which has a lower reactivity is esterified more slowly than the remainder of the cellulosic material in said batch. To insure the esterification of the least reactive cellulosic material in a batch, the esterification time must be lengthened considerably, further reducing the capacity of the esterification equipment and increasing the esterification cost.

It is an important object of this invention to provide a process for the preparation of organic acid esters of cellulose which will be free from

the foregoing and other disadvantages of the processes previously used for this purpose.

A further object of this invention is to provide a process for treating cellulosic material that is to be employed for the production of organic acid esters of cellulose so that different batches of cellulosic material from a given source will have substantially the same reactivity after pretreatment.

Another object of this invention is to provide a process for treating cellulosic material that is to be employed for the production of organic acid esters of cellulose so that all the cellulosic material in a single batch will have substantially the same reactivity after pretreatment.

A still further object of this invention is to provide a process for treating cellulosic material that is to be employed for the production of organic acid esters of cellulose so that the cellulosic material will have a higher reactivity after pretreatment.

Other objects of this invention will be apparent from the following detailed description and claims.

25 It has been found that the variations, after pretreatment, in the reactivity of different batches of cellulosic material from a given source and in different portions of a single batch of cellulosic material are the result of differences

30 both in moisture content of the cellulosic material immediately prior to pretreatment and in the "moisture history" of said cellulosic material. Thus, as the moisture content of the cellulosic material falls below about 5% by weight, there is a corresponding decrease in the reactivity of said cellulosic material after pretreatment.

35 When the moisture content of the cellulosic material falls further to below about 4% by weight there is an accelerated decrease in the reactivity of the cellulosic material after pretreatment so that when the moisture content of the cellulosic material falls to below about 3% by weight, the pretreatment has substantially no effect on the reactivity of the cellulosic material.

40 The phrase "cellulosic material from a given source" employed herein denotes cellulosic material derived from a single type of plant such as cotton linters, wood pulp, etc. that has been purified by the same process.

45 Another factor that determines the reactivity of the cellulosic material after pretreatment is the "moisture history" of the cellulosic material. For example, if a batch of cellulosic material having a given moisture content is pretreated, its reactivity after pretreatment will depend upon

whether the moisture content of said cellulosic material has previously been below about 5% by weight. A cellulosic material whose moisture content has not been below said value will have a higher reactivity after pretreatment than will a cellulosic material whose moisture content had dropped below said value and then been raised to said value before pretreatment. This difference in the reactivity of the cellulosic material after pretreatment is particularly marked when the moisture content of the cellulosic material falls to less than about 1% by weight before pretreatment and is subsequently raised to a higher value. Since both the moisture content and the "moisture history" of different batches of cellulosic material from a given source or in different portions of a single batch of cellulosic material may vary as the result of variations in conditions during the production and storage of said cellulosic material, there is a considerable variation in the reactivity of the cellulosic material after pretreatment.

According to the present invention, we have discovered that the variations, after pretreatment, in the reactivity of different batches of cellulosic material from a given source and in different portions of a single batch of cellulosic material may be eliminated by bringing the moisture content of said cellulosic material to at least about 15% by weight, and evaporating at least about 5% or preferably at least about 10% by weight of water on the weight of the cellulosic material from the cellulosic material without, however, reducing the moisture content of the cellulosic material to less than about 4.5% or preferably less than about 5% by weight. Upon pretreatment of cellulosic material that has been treated in this manner, there is obtained a product having a uniform reactivity both as between different batches of cellulosic material from a given source and as between different portions of a single batch of cellulosic material. The process of this invention is especially advantageous in treating cellulosic material whose moisture content had dropped below about 1% by weight since this cellulosic material is extremely resistant to activation during the pretreatment process.

In carrying out the treatment of this invention a sufficient quantity of moisture is added to the cellulosic material to bring the moisture content of said material to at least about 15% by weight, or, advantageously, to between about 15 and 30% by weight. The addition of a greater quantity of water to the cellulosic material will not make the reactivity of the cellulosic material, after pretreatment, less uniform. However, the addition of this greater quantity of water is relatively undesirable, when the water is added simply to make more uniform the reactivity of the cellulosic material after pretreatment, since the additional water must either be evaporated from the cellulosic material or, if permitted to remain in the cellulosic material, it will react with the organic acid anhydride employed in the esterification medium, converting the same to the corresponding organic acid.

The water should be distributed through the cellulosic material in such fashion that the moisture content of substantially all the cellulosic material is raised to at least about 15% by weight. To this end, the water may be sprayed onto a mass of cellulosic fibers and the mixture stirred thoroughly until the desired distribution has been effected. After the moisture content of the cellulosic material has been adjusted to the de-

sired value, at least about 5% or preferably at least about 10% by weight of water is evaporated from the cellulosic material without, however, permitting the moisture content of the cellulosic material to fall below about 4.5% or preferably below about 5% by weight. Preferably a sufficient quantity of water is evaporated from the cellulosic material to reduce its moisture content to between about 5 and 7% by weight, since, if a larger quantity of water is permitted to remain in the cellulosic material, the additional water will react with the organic acid anhydride employed for the esterification, converting the same to the corresponding organic acid. The evaporation of the water from the cellulosic material may be effected rapidly by blowing an evaporative medium such as air through said material. The evaporative medium may be heated to a temperature of between about 25 and 65° C., or more, if desired, to increase the rate of evaporation. Care should be taken, in this case, to avoid over-drying any portions of the cellulosic material, since overdrying will both reduce and make non-uniform the reactivity, after pretreatment, of the cellulosic material.

The addition of water to the cellulosic material and the subsequent evaporation of the water therefrom can be carried out very rapidly. Thus, the addition of water to the cellulosic material can be effected, with agitation, in as little as about 10 seconds or in from about 10 to 60 seconds, while the evaporation of the water from the cellulosic material can be effected in as little as about 50 seconds or in from about 50 to 150 seconds. Although longer periods of time may be employed both for adding the water to the cellulosic material and for evaporating the water therefrom without impairing the reactivity of the cellulosic material after pretreatment, these longer periods are somewhat less desirable as they are not as efficient in the use of equipment. The rapidity with which the treatment of this invention can be carried out makes it applicable to both batch and continuous esterification processes.

By bringing the moisture content of the cellulosic material to at least about 90% by weight, or, advantageously, to between about 90 and 100% by weight, before evaporating the water therefrom, it is possible, in certain cases, not only to make more uniform, but also to increase considerably the reactivity of the cellulosic material after pretreatment. In this case, at least about 80% by weight of water is evaporated from the cellulosic material before the pretreatment, without, however, permitting the moisture content to fall below about 4.5% or preferably below about 5% by weight.

Following the evaporation of the water, the cellulosic material is pretreated to increase its reactivity in a manner well known in the art. For example, the cellulosic material may be treated with a lower aliphatic acid such as formic, acetic or propionic acid, or mixtures thereof, or the like and containing, if desired, a small proportion of an esterification catalyst such as phosphoric or sulfuric acid. The cellulosic material may also be pretreated in accordance with the multi-stage process described in Seymour et al., U. S. application No. 58,028, filed November 2, 1948. The pretreated cellulosic material is then esterified with an organic acid anhydride in a manner well known in the art, preferably in the presence of an esterification catalyst and an organic acid which acts as a solvent for the cellulose ester being formed.

The cellulosic material that has been treated in accordance with this invention exhibits a substantially uniform reactivity, after pretreatment, both as between different batches of cellulosic material from a given source and as between different portions of a single batch of cellulosic material as evidenced by the reproducibility of the time required to complete the esterification. Moreover, when the moisture content of the cellulosic material has been raised to above about 90% by weight, it exhibits, in certain cases, not only a more uniform reactivity after pretreatment, but also a greatly increased reactivity after pretreatment, thereby permitting the esterification time with a given esterification process to be reduced up to about 30% or even more.

The moisture content of the cellulosic material as set forth herein is measured on the dry weight of the cellulosic material, i. e. a cellulosic material having a moisture content of 5% by weight contains 5 parts by weight of water for every 100 parts by weight of the dry cellulosic material.

The process of the present invention may be applied to any suitable cellulosic material, such as cotton linters, or wood pulps or the like from which the major portion of the lignin, pentosans, resins and similar constituents have been removed, as, for example, purified sulfite pulp, sulfate pulp or soda pulp. In addition, there may be employed cellulosic material derived from other sources such as bamboo, reeds, jute, esparto, straws, such as linseed and hempseed straw, grasses, peanut hulls, bark, etc. The cellulosic material is advantageously pretreated in the form of a mass of loose fibers to permit ready access of the added water to all portions of the fibers and to permit the water to be evaporated uniformly from the fibers.

While our invention will be especially described in connection with the preparation of cellulose acetate, it is to be understood that it is also applicable to the preparation of other organic acid esters of cellulose such as the simple and mixed lower aliphatic acid esters of cellulose including cellulose propionate, cellulose butyrate, cellulose acetate-propionate, cellulose acetate-butyrate and the like. In addition, it is applicable to the preparation of other organic acid esters of cellulose such as cellulose acetate stearate, as well as to the benzoic acid ester of cellulose.

The following examples are given to illustrate the invention further:

#### Example I

Cotton linters having a moisture content of 5.74% by weight are oven dried for 2 hours at 100° C., reducing their moisture content to 0.24% by weight. Portions of both the oven dried and the undried cotton linters are separately pretreated by adding to 60 parts by weight of the cotton linters, 21 parts by weight of glacial acetic acid containing 0.3 parts by weight of sulfuric acid and agitating the mixture so formed for 2 hours. The pretreated cotton linters are cooled to 3 to 8° C. and esterified by treatment with a mix cooled to 3 to 5° C. and containing 399 parts by weight of glacial acetic acid, 177 parts by weight of acetic anhydride and 7.6 parts by weight of sulfuric acid. The time required to complete the esterification of the undried cotton linters, as evidenced by the clearing of the esterification medium, is 25 minutes whereas the dried cotton linters are not fully esterified after 45 minutes, an increase in esterification time of more than 80%.

#### Example II

A sample of the dried cotton linters produced in Example I is mixed for 19 hours with sufficient water to bring its moisture content up to 5.76% by weight. The cotton linters are then pretreated and esterified in the manner set forth in Example I. The time required to complete the esterification of the cotton linters treated in this manner is 20% greater than the time required to esterify the cotton linters that have not been dried, showing that the cotton linters have not regained their original reactivity although their moisture content has been restored to substantially its original value.

#### Example III

A sample of the dried cotton linters produced in Example I is mixed for 10 seconds with 15.9% by weight of water and is then dried to a moisture content of 5.61% by weight by blowing air heated to a temperature of 62° C. through the cotton linters for 50 seconds. The cotton linters are then pretreated and esterified in the manner set forth in Example I. The time required to complete the esterification of the cotton linters treated in this manner is substantially the same as that required to esterify the cotton linters that have not been dried, showing that the cotton linters have regained their original reactivity although their moisture content is somewhat lower than its original value.

#### Example IV

Cotton linters having a moisture content of 5.92% by weight are mixed for 20 seconds with 87.9% by weight of water and are then dried to a moisture content of 6.10% by weight by blowing air heated to a temperature of 45.5° C. through the cotton linters for 9 minutes. The cotton linters are then pretreated and esterified in the manner set forth in Example I. The time required to complete the esterification of the cotton linters treated in this manner is 27% less than that required to esterify the untreated cotton linters, showing that the cotton linters have an increased reactivity.

It is to be understood that the foregoing detailed description is given merely by way of illustration and that many variations may be made therein without departing from the spirit of our invention.

Having described our invention, what we desire to secure by Letters Patent is:

1. In a process for the production of lower aliphatic acid esters of cellulose by the esterification of a cellulosic material, the steps of increasing the activity of cellulosic material by adding moisture to cellulosic material in the form of a mass of loose fibers, which cellulosic material without said additional moisture would not have its reactivity increased, to bring the moisture content of the cellulosic material to at least about 15% by weight, evaporating from the cellulosic material at least about 5% by weight of moisture on the weight of the cellulosic material without reducing the moisture content of the cellulosic material to less than about 4.5% by weight, pretreating the cellulosic material by adding a lower aliphatic acid thereto without displacing the moisture contained therein, and esterifying the pretreated cellulosic material with a lower aliphatic acid anhydride.

2. In a process for the production of lower aliphatic acid esters of cellulose by the esterification of a cellulosic material, the steps of in-

creasing the activity of cellulosic material by adding moisture to cellulosic material in the form of a mass of loose fibers, which cellulosic material without said additional moisture would not have its reactivity increased, to bring the moisture content of the cellulosic material to at least about 15% by weight, evaporating from the cellulosic material at least about 10% by weight of moisture on the weight of the cellulosic material without reducing the moisture content of the cellulosic material to less than about 5% by weight, pretreating the cellulosic material by adding a lower aliphatic acid thereto without displacing the moisture contained therein, and esterifying the pretreated cellulosic material with a lower aliphatic acid anhydride.

3. In a process for the production of lower aliphatic acid esters of cellulose by the esterification of a cellulosic material, the steps of increasing the activity of cellulosic material by adding moisture to cellulosic material in the form of a mass of loose fibers, which cellulosic material without said additional moisture would not have its reactivity increased, to bring the moisture content of the cellulosic material to between about 15 and 30% by weight, evaporating from the cellulosic material sufficient moisture to bring the moisture content of the cellulosic material to between about 5 and 7% by weight, pretreating the cellulosic material by adding a lower aliphatic acid thereto without displacing the moisture contained therein, and esterifying the pretreated cellulosic material with a lower aliphatic acid anhydride.

4. In a process for the production of lower aliphatic acid esters of cellulose by the esterification of a cellulosic material, the steps which comprise adding moisture to cellulosic material in the form of a mass of loose fibers to bring the moisture content of the cellulosic material to at least about 90% by weight, evaporating from the cellulosic material at least about 80% by weight of moisture on the weight of the cellulosic material without reducing the moisture content of the cellulosic material to less than about 4.5% by weight, pretreating the cellulosic material by adding a lower aliphatic acid thereto without displacing the moisture contained therein, and esterifying the pretreated cellulosic material with a lower aliphatic acid anhydride.

5. In a process for the production of lower aliphatic acid esters of cellulose by the esterification of a cellulosic material, the steps which comprise adding moisture to cellulosic material in the form of a mass of loose fibers to bring the moisture content of the cellulosic material to between about 90 and 100% by weight, evaporating from the cellulosic material sufficient moisture to bring the moisture content of the cellulosic material to between about 5 and 7% by weight, pretreating the cellulosic material by adding a lower aliphatic acid thereto without displacing the moisture contained therein, and esterifying the pretreated cellulosic material with a lower aliphatic acid anhydride.

6. In a process for the production of lower aliphatic acid esters of cellulose by the esterification of a cellulosic material, the steps of increasing the activity of cellulosic material by adding moisture to cellulosic material in the form of a mass of loose fibers, which cellulosic material without said additional moisture would not have its reactivity increased, to bring the moisture content of the cellulosic material to at least about 15% by weight, passing air hav-

ing a temperature of between about 25 and 65° C. through the cellulosic material to evaporate from the cellulosic material at least about 5% by weight of moisture on the weight of the cellulosic material without reducing the moisture content of the cellulosic material to less than about 4.5% by weight, pretreating the cellulosic material by adding a lower aliphatic acid thereto without displacing the moisture contained therein, and esterifying the pretreated cellulosic material with a lower aliphatic acid anhydride.

7. In a process for the production of lower aliphatic acid esters of cellulose by the esterification of a cellulosic material, the steps of increasing the activity of cellulosic material by adding moisture to cellulosic material in the form of a mass of loose fibers, which cellulosic material without said additional moisture would not have its reactivity increased, in a period of from about 10 to 60 seconds to bring the moisture content of the cellulosic material to at least about 15% by weight, evaporating from the cellulosic material at least about 5% by weight of moisture on the weight of the cellulosic material in a period of from about 50 to 150 seconds without reducing the moisture content of the cellulosic material to less than about 4.5% by weight, pretreating the cellulosic material by adding a lower aliphatic acid thereto without displacing the moisture contained therein, and esterifying the pretreated cellulosic material with a lower aliphatic acid anhydride.

8. In a process for the production of lower aliphatic acid esters of cellulose by the esterification of a cellulosic material, the steps which comprise adding moisture to cellulosic material in the form of a mass of loose fibers and having a moisture content of less than 1% by weight to bring the moisture content of the cellulosic material to at least about 15% by weight, evaporating from the cellulosic material at least about 5% by weight of moisture on the weight of the cellulosic material without reducing the moisture content of the cellulosic material to less than about 4.5% by weight, pretreating the cellulosic material by adding a lower aliphatic acid thereto without displacing the moisture contained therein, and esterifying the pretreated cellulosic material with a lower aliphatic acid anhydride.

9. In a process for the production of cellulose acetate by the acetylation of a cellulosic material, the steps of increasing the activity of cellulosic material by adding moisture to cellulosic material in the form of a mass of loose fibers, which cellulosic material without said additional moisture would not have its reactivity increased, to bring the moisture content of the cellulosic material to at least about 15% by weight, evaporating from the cellulosic material at least about 5% by weight of moisture on the weight of the cellulosic material without reducing the moisture content of the cellulosic material to less than about 4.5% by weight, pretreating the cellulosic material by adding a lower aliphatic acid thereto without displacing the moisture contained therein, and acetylating the pretreated cellulosic material with acetic anhydride.

10. In a process for the production of cellulose acetate by the acetylation of a cellulosic material, the steps of increasing the activity of cellulosic material by adding moisture to cellulosic material in the form of a mass of loose fibers, which cellulosic material without said additional moisture would not have its reactivity

increased, to bring the moisture content of the cellulosic material to at least about 15% by weight, evaporating from the cellulosic material at least about 10% by weight of moisture on the weight of the cellulosic material without reducing the moisture content of the cellulosic material to less than about 5% by weight, pretreating the cellulosic material by adding a lower aliphatic acid thereto without displacing the moisture contained therein, and acetylating the pretreated cellulosic material with acetic anhydride.

11. In a process for the production of cellulose acetate by the acetylation of a cellulosic material, the steps of increasing the activity of cellulosic material by adding moisture to cellulosic material in the form of a mass of loose fibers, which cellulosic material without said additional moisture would not have its reactivity increased, to bring the moisture content of the cellulosic material to between about 15 and 30% by weight, evaporating from the cellulosic material sufficient moisture to bring the moisture content of the cellulosic material to between about 5 and 7% by weight, pretreating the cellulosic material by adding a lower aliphatic acid thereto without displacing the moisture contained therein and an esterification catalyst, and acetylating the pretreated cellulosic material with acetic anhydride.

12. In a process for the production of cellulose acetate by the acetylation of a cellulosic material, the steps which comprise adding moisture to cellulosic material in the form of a mass of loose fibers to bring the moisture content of the cellulosic material to at least about 90% by weight, evaporating from the cellulosic material at least about 80% by weight of moisture on the weight of the cellulosic material without reducing the moisture content of the cellulosic material to less than about 4.5% by weight, pretreating the cellulosic material by adding a lower aliphatic acid thereto without displacing the moisture contained therein, and acetylating the pretreated cellulosic material 45 with acetic anhydride.

13. In a process for the production of cellulose acetate by the acetylation of a cellulosic material, the steps which comprise adding moisture to cellulosic material in the form of a mass of loose fibers to bring the moisture content of the cellulosic material to between about 90 and 100% by weight, evaporating from the cellulosic material sufficient moisture to bring the moisture content of the cellulosic material to between about 5 and 7% by weight, pretreating the cellulosic material by adding a lower aliphatic acid thereto without displacing the moisture contained therein and an esterification catalyst, and acetylating the pretreated cellulosic material with acetic anhydride.

PETER BLACKMAN.

FRED FORTRESS.

BLANCHE B. WHITE.

#### REFERENCES CITED

The following references are of record in the file of this patent:

#### UNITED STATES PATENTS

|    | Number    | Name           | Date          |
|----|-----------|----------------|---------------|
| 25 | 1,543,310 | Altwegg        | June 23, 1925 |
|    | 2,063,324 | Malm et al.    | Dec. 8, 1936  |
|    | 2,087,263 | Olsen          | July 20, 1937 |
|    | 2,105,498 | Parrett et al. | Jan. 18, 1938 |
| 30 | 2,113,301 | Gardner        | Apr. 5, 1938  |
|    | 2,119,117 | Schuller       | May 31, 1938  |
|    | 2,345,406 | Malm           | Mar. 28, 1944 |
|    | 2,478,396 | Hincke et al.  | Aug. 9, 1949  |
| 35 | 2,484,455 | Herdle et al.  | Oct. 11, 1949 |
|    | 2,487,892 | Richter et al. | Nov. 15, 1949 |
|    | 2,490,754 | Hincke et al.  | Dec. 6, 1949  |

#### FOREIGN PATENTS

|    | Number  | Country       | Date |
|----|---------|---------------|------|
| 40 | 491,583 | Great Britain | 1938 |

#### OTHER REFERENCES

Worden, "Technology of Cellulose Esters," vol. 8, 1916, page 2567.